

Patented Dec. 7, 1943

2,336,340

# UNITED STATES PATENT OFFICE

2,336,340

## STABILIZATION OF CELLULOSIC FABRICS

Louis H. Bock, Huntingdon Valley, and Alva L. Houk, Philadelphia, Pa., assignors to Röhm & Haas Company, Philadelphia, Pa., a corporation of Delaware

No Drawing. Application December 28, 1940,  
Serial No. 372,166

4 Claims. (Cl. 8—120)

This invention relates to a method for stabilizing cellulosic fabrics against changes in dimensions by a reaction between the fabric and a compound of the formula



wherein R is an aliphatic group containing two to ten carbon atoms, R<sub>1</sub> is a group containing less than 12 carbon atoms selected from the class consisting of aliphatic, alicyclic hydrocarbon and aralkyl groups, R<sub>2</sub> and R<sub>3</sub> when taken individually are members of the class consisting of aliphatic hydrocarbon groups of one to four carbon atoms and when taken together are saturated divalent groups which jointly with the nitrogen form a heterocycle, and X is a salt-forming anion.

Shrinkage control has heretofore been attained by mechanical treatment of cotton cloth or by the use of resins. Mechanical treatment does not, however, protect against stretching in a subsequent operation, while the resins which have been found effective impart to the cloth properties which are often undesirable.

It is an object of this invention to render fabrics composed of cotton, linen, rayon, or other cellulosic fibers resistant to shrinking or stretching. It is also an object to thus stabilize fabrics while preserving appearance and handle of the original fabric. It is a further object to stabilize cellulosic fabrics without having to incorporate therein resins or deposits of nitrogenous materials.

These objects are accomplished by impregnating cellulosic fabrics with a solution containing at least about 5% of a quaternary ammonium salt of the above general formula and preferably not more than 15% of said salt and heating the impregnated fabric while holding it at desired dimensions until reaction between fabric and compound takes place. In the reaction a methyl ether group from the compound combines with cellulose to form a new compound and the amine portion of the quaternary compound is split out and eliminated from the fabric by volatilization, by washing, or by other suitable procedure. The process is performed with optimum stabilization and yield of fabric when the impregnated fabric is at the desired finished dimensions during the reaction. These dimensions may preferably be attained during the stage when drying takes place. Drying may be performed at low or high temperature, either as a separate step or incidental to the heating of the impregnated fabric.

Typical of the quaternary ammonium salts which are useful in this invention are the following: di-ethyloxymethyl dimethyl ammonium chloride, butoxymethyl methoxymethyl dimethyl ammonium bromide, hexyloxymethyl propyloxymethyl diethyl ammonium chloride, octyloxymethyl

methyl butoxymethyl methyl butyl ammonium bromide, amyloxyethyl undecenyloxymethyl dimethyl ammonium chloride, butoxymethyl cyclohexyloxymethyl dimethyl ammonium chloride, butoxymethyl allyloxyethyl dimethyl ammonium chloride, butoxymethyl benzyloxymethyl diethyl ammonium chloride, capryloxyethyl isopropoxymethyl dimethyl ammonium chloride, di-butoxyethyl morpholinium chloride, butoxymethyl ethoxymethyl pyrrolidinium bromide, butoxymethyl ethoxymethyl piperidinium bromide, phenoxyethoxymethyl ethoxymethyl dimethyl ammonium bromide, or the like. The halogens in the above compounds may be replaced with other anions, such as acetate, formate, sulfate, etc. The compounds having R—O—CH<sub>2</sub>— groups containing four carbon atoms in the group designated by R or R<sub>1</sub> have been found to give the optimum degree of stabilization. The effect clearly persists, however, up to a chain of 12 carbon atoms. Very long groups may have an opposite effect, probably because of their lubricating action. The presence of two methyl ether groups in the quaternary ammonium salt renders these compounds peculiarly effective in stabilizing cellulose fabrics. They react under conditions which give the desired effects without causing undue tendering of the fabric or change in its original appearance and handle.

The fabrics which have been improved in stability as to dimensions include those woven from cotton, linen, regenerated cellulose of the several types, etc., and those prepared from mixtures of these cellulosic materials.

The stabilization of fabrics is illustrated in the following examples:

### Example 1

A piece of an 80 x 80, 4 yd. 36 in. cotton sheeting was impregnated with a 10% aqueous solution of 2-ethylhexyloxymethyl benzyloxymethyl dimethyl ammonium chloride. The cloth was then held within desired dimensions by clamping in a rigid frame, whereupon it was dried at room temperature, and heated for 30 minutes in an oven at 130° C. The cloth was removed from the frame, carefully measured, laundered in a hot solution of soap and soda ash, rinsed, dried, and ironed. The dimensions of the piece were determined and the shrinkage found to be 2.6% in the warp.

A piece of the original cloth not treated with the quaternary ammonium salt, was measured, laundered in the same soap bath, rinsed, dried, and ironed. It shrank 5.25% along the warp.

### Example 2

A piece of 80 x 80, 4 yd. 36 in. cotton sheeting was held within desired dimensions by clamping in a frame and while so held it was impregnated

with a 10% aqueous solution of isoamyloxy-methyl isopropoxy-methyl dimethyl ammonium chloride, and thereafter freed of excess solution, dried at 30° C., heated in an oven at 130° C. for one-half hour, and removed from the frame. Pieces of cloth were marked, carefully measured, washed in a hot solution of soap and soda ash, rinsed, dried, and ironed. Shrinkage along the warp was only 1.9%.

*Example 3*

Other pieces of the same cotton sheeting as used in the foregoing examples were impregnated in a 5% aqueous solution of di-butoxymethyl dimethyl ammonium chloride, placed on a frame, dried under tension for five minutes in an oven at 130° C., and heated for ten minutes in an oven at 150° C. The pieces were removed from the frame, measured, and laundered as above. Shrinkage along the warp was 1.8%.

Other pieces of the sheeting were treated by the same procedure with substitution of a 10% aqueous solution for the 5% solution of the same compound. Shrinkage was 0.9%.

Still other pieces were impregnated with di-butoxymethyl dimethyl ammonium chloride, stretched in a frame, and placed in an oven at 150° C. for five minutes. These pieces, after being laundered, shrank 1.9% along the warp.

*Example 4*

A piece of dyed 39 inch, 58 x 68, 3.4 yds. per lb., spun rayon slab was clamped in a rigid frame and impregnated with a 10% aqueous solution of dibutoxymethyl dimethyl ammonium chloride. It was dried at room temperature and then placed in an oven at 130° C. for 30 minutes. The cloth was then removed from the frame and carefully measured. It was then laundered and treated as in Example No. 1. The shrinkage was 0.6% in the direction of the warp; the shrinkage of the original sheet under the same treatment was 1.5%.

*Example 5*

A piece of 33 inch, 68 x 62, 3.5 yards per lb., all-spun bright viscose rayon challis, 1.5 denier, 1 $\frac{1}{2}$  inch staple was clamped in a frame impregnated with an aqueous solution containing 12% of dibutoxymethyl dimethyl ammonium chloride and 2% ammonium chloride. The impregnated fabric was air-dried, and placed in an oven at 130° C. for 30 minutes. The cloth was removed from the frame and carefully measured. It was then laundered in a hot solution of soap and soda ash, rinsed, dried and ironed. The shrinkage was now found to be 3.1% in the warp whereas the original fabric shrank 7.5%. In this case shrinkage in the filling was also determined as 0.6% in the treated piece and 3.9% in the original fabric.

We claim:

1. A process for stabilizing cellulosic fabrics against changes in dimensions, which comprises impregnating said fabrics with a solution containing between about 5% and about 15% of a quaternary compound of the formula



wherein R is an aliphatic group containing two

to ten carbon atoms, R<sub>1</sub> is a group containing less than twelve carbon atoms selected from the class consisting of aliphatic, alicyclic hydrocarbon and aralkyl groups, R<sub>2</sub> and R<sub>3</sub> when taken individually are members of the class consisting of aliphatic hydrocarbon groups of one to four carbon atoms and when taken together are saturated divalent groups which jointly with the nitrogen form a heterocycle, and X is a salt-forming anion, drying the impregnated fabric under conditions imparting the desired dimensions, heating to cause reaction between fabric and compound, and eliminating nitrogenous compounds.

2. A process for stabilizing cellulosic fabrics against changes in dimensions, which comprises impregnating said fabrics with a solution containing between about 5% and about 15% of a quaternary ammonium salt of the formula



wherein R is an aliphatic group containing two to ten carbon atoms, R<sub>1</sub> is a group containing less than twelve carbon atoms selected from the class consisting of aliphatic, alicyclic hydrocarbon, and aralkyl groups, R<sub>2</sub> and R<sub>3</sub> when taken individually are members of the class consisting of aliphatic hydrocarbon groups of one to four carbon atoms and when taken together are saturated divalent groups which jointly with the nitrogen form a heterocycle, and X is a salt-forming anion, heating the impregnated fabric to a temperature between about 100° C. and 150° C. while maintaining the fabric at desired finished dimensions, and washing the treated fabric.

3. A process for stabilizing cellulosic fabrics against changes in dimensions, which comprises impregnating said fabrics with a solution containing between about 5% and about 15% of a quaternary ammonium salt of the formula



wherein R is an aliphatic hydrocarbon group having four carbon atoms, R<sub>1</sub>, R<sub>2</sub>, and R<sub>3</sub> are aliphatic hydrocarbon groups of less than five carbon atoms, and X is a halogen, drying the impregnated fabric while maintaining the fabric at desired finished dimensions, and heating the fabric to cause reaction between fabric and quaternary salt.

4. A process for stabilizing cellulosic fabrics against changes in dimensions, which comprises impregnating said fabrics with a solution containing between about 5% and about 15% of a quaternary ammonium salt of the formula



wherein X is a halogen, drying the impregnated fabric at the desired finished dimensions in a tenter and heating the dried fabric between about 100° C. and about 150° C.